

Feb. 20, 1962

R. A. HACKLEY ETAL

3,022,195

FERROSPINEL BODY HAVING INTEGRAL METALLIC SURFACE LAYER

Original Filed Nov. 18, 1953



INVENTORS.  
REGINALD A. HACKLEY &  
ROBERT L. HARVEY  
By  
W.S. /file  
AGENT

# United States Patent Office

3,022,195

Patented Feb. 20, 1962

1

3,022,195

## FERROSPINEL BODY HAVING INTEGRAL METALLIC SURFACE LAYER

Reginald A. Hackley and Robert L. Harvey, Princeton, N.J., assignors to Radio Corporation of America, a corporation of Delaware

Original application Nov. 18, 1953, Ser. No. 392,848, now Patent No. 2,957,238, dated Oct. 25, 1960. Divided and this application Dec. 22, 1959, Ser. No. 861,360  
7 Claims. (Cl. 117—123)

This is a division of U.S. application 392,848, now U.S. Patent No. 2,957,238, filed November 18, 1953, by Robert L. Harvey and Reginald A. Hackley and assigned to the same assignee as the assignee of this divisional application.

This invention relates to methods of forming metallic surface layers on ferrospinel bodies and more particularly to forming such layers integrally united to said bodies.

The coined word ferrospinel is used herein to denote a ferromagnetic spinel, which is a species of non-metallic, cubic crystalline material containing iron in chemically combined form. The term ferrospinel seems doubly appropriate because the materials use chiefly the spin property of unpaired electrons. Ferrospinel are sometimes called ferrites, a term which is also used to denote a form of metallic iron containing a fraction of a percent of carbon. The definition of ferrospinel as defined herein is also defined in the same manner in the RCA Review article cited below, vol. 11, page 321, footnote.

Ferrospinel bodies, also known as ferrites, are well known and have been found especially useful because of their magnetic properties. Ferrospinel are unique crystalline materials of spinel structure which are formed at relatively high temperatures by solid-phase reaction of iron oxide and one or more of other metallic oxides.

Certain ferrospinel exhibit relatively pronounced magnetostrictive properties and are especially useful in transducer devices because of their low eddy current losses and relatively high efficiencies. See, for example, an article in the RCA Review, volume 11, September 1950, entitled "Ferromagnetic Spinel for Radio Frequencies," pages 321 to 362.

In certain forms of magnetostrictive transducers, it is desirable to transfer vibrational energy from a ferrospinel body to another body which is usually metallic. To effect efficient energy transfer it is desirable to provide a rigid, relatively noncompliant connection between the ferrospinel and the magnetic bodies.

Difficulty has been encountered in attempting to fasten ferrospinel bodies to metallic bodies. Various cements have been utilized and attempts have been made to solder a ferrospinel body to a metallic member. Cement films, however, tend to fail when subjected to vibrational forces. It has not previously been possible satisfactorily to bond a ferrospinel body to a metallic surface by a solder connection principally because of the difficulty of making solder adhere to the body.

Accordingly one object of the instant invention is to provide a ferrospinel body having a surface layer of a metal integrally united with the body.

This and other objects may be accomplished by the practice of the instant invention according to which a surface portion of a ferrospinel body is chemically reduced to provide a metal surface integrally united with the body.

The invention will be described in greater detail with reference to the drawing of which the single figure is a schematic, vertical, cross-sectional view of a ferrospinel body soldered to a metallic base according to the invention.

According to a preferred embodiment of the invention a metallic surface layer may be produced upon the surface

2

of a ferrospinel body as shown in the drawing. A ferrospinel body consisting essentially of  $\text{NiFe}_2\text{O}_4$  is heated for about one minute by a hydrogen torch. The torch is fed with hydrogen only in order to provide an incompletely combusted flame. The temperature of the surface is raised preferably to about 1000° F. The excess hydrogen of the flame reduces a surface portion of the body to a metal which is believed to be an alloy of iron and the other metals of the oxides.

Unexpectedly, the metallic surface portion produced by the reduction is cohesive, relatively smooth and very strongly adherent to the oxide body. Ordinarily it would be expected that a reduction process would produce a granular or flaky, non-adherent layer of metal. It has been found, however, that in the case of a ferrospinel, such a reduced surface layer or portion is continuous and inseparably bonded to the ferrospinel body. It is believed that the adherence of the metal to the ferrospinel is at least partially due to an interlocking of the crystalline structures of the respective materials. It is thought that the reduction process, while completed at the surface and for a short distance beneath the surface, extends in an increasingly incomplete form some distance into the ferrospinel composition.

The thickness of the metal surface layer may be readily controlled by varying the time and the temperature of heating as described heretofore. Heating for a longer time or at a hotter temperature or both produces a relatively thick metal layer. Heating for a relatively short time, such as a few seconds, or at a relatively low temperature tends to produce a relatively thin metallic layer.

The practice of the instant invention is equally applicable to produce metallic surface layers on ferrospinel compositions other than the  $\text{NiFe}_2\text{O}_4$  heretofore described. For example, methods exactly similar to those described herein may be utilized to produce a metallic surface layer on bodies of any of the ferrospinel compositions described in the RCA Review article referred to, such as compositions comprising  $\text{Fe}_2\text{O}_3$  in solid solution with  $\text{CuO}$ ,  $\text{Mn}_3\text{O}_4$ ,  $\text{ZnO}$ ,  $\text{NiO}$  and mixtures of these oxides. The method is generally applicable to all ferrospinel materials.

The upper temperature limit that may be conveniently utilized to form the metallic surface layer on a ferrospinel body is primarily determined by the temperature tolerance of the ferrospinel composition. Many ferrospinel bodies, especially relatively large ones, are apt to crack or to break apart when subjected to unbalanced heating such as is produced by heating one surface only. In general, the temperature utilized is preferably not higher than about 1800° F.

The minimum operating temperature is the minimum temperature at which reduction can be made to take place at a reasonably rapid rate, about 750° F. Somewhat higher temperatures are preferred, however, because of the relative increase in speed of reduction and the shorter time required.

In many instances, relatively large bodies of ferrospinel composition cannot be readily treated as described heretofore without damage by thermal shock. In these cases, and generally in the cases of ferrospinel bodies having a minimum cross-sectional dimension of  $1/4$ " and greater, it has been found more satisfactory and convenient to reduce a surface portion of the body by other means. Such relatively large ferrospinel bodies may be treated according to the invention by heating them uniformly in a hydrogen furnace, that is, in a furnace having means to maintain the body in a hydrogen-rich atmosphere. The ferrospinel bodies may be heated in a hydrogen atmosphere for about one hour at about 1300° F. and allowed to cool in a hydrogen atmosphere. This heating produces a metallic surface layer on the ferrospinel body over all its ex-

posed surface. If it is desired to provide only a portion of the ferrospinel surface with a metallic layer, suitable masking means such as a quartz powder may be applied to the surface of the body. Alternatively, a metallic surface layer may be produced over the entire surface of the body and unwanted portions of the layers may be removed by etching in a dilute acid such as sulphuric or muriatic acid.

Instead of heating the ferrospinel body in the presence of hydrogen, the body alternatively may be heated to about the same temperatures in the presence of carbon to produce essentially the same results.

The temperature limitations for this embodiment of the invention are about the same as those heretofore set forth. The time required, however, is somewhat longer. Depending on the temperature and on the desired thickness of the metal layer, furnace heating may be for a few minutes up to two or more hours.

A ferrospinel body having a metallic surface layer produced according to any of the methods heretofore described may be readily soldered to a metallic body as shown in the drawing. A ferrospinel body 2 having a metallic surface layer 4 produced according to the instant invention is securely soldered to a metal base 10 by a solder joint 8. Previously to soldering, the metallic surface layer is preferably buffed or polished using steel wool or any convenient abrasive to produce a bright, smooth finish. Any conventional soldering material and flux suitable for soldering to iron may be used such as silver solder and zinc chloride. In the case of relatively large ferrospinel bodies, however, it is preferred to use a relatively low melting point solder such as a solder composed of 50% tin and 50% lead in order to avoid excessive thermal strains within the bodies which may serve to weaken or even to crack them.

The practice of the instant invention is, of course, not limited to bodies made of ferrospinel compositions having especially pronounced magnetostrictive properties but is equally applicable to all known ferrospinel.

What is claimed:

1. A ferrospinel body having a metallic layer on a surface portion thereof, said layer having been derived from said body and being an integral part thereof.

2. A ferrospinel body containing iron in chemically combined form and having a metallic layer on a surface portion thereof, said metallic layer having been derived from said body by the chemical reduction of a surface portion of said body, said metallic layer being an integral part of said body.

3. A ferrospinel body comprising a sintered crystalline product including iron in chemically combined form, said body having metallic layer integral with a surface portion thereof, said surface portion having been produced by the chemical reduction of a surface portion of said body.

4. A ferrospinel body comprising a sintered crystalline product including ferric oxide and at least one other metallic oxide in chemically combined form, said body having a metallic layer integral with a surface portion thereof, said metallic layer consisting essentially of the metals of said oxides and having been derived from said body by the chemical reduction of a surface portion of said body.

5. A ferrospinel body comprising a sintered crystalline product including ferric oxide and at least one other metallic oxide and having a spinel structure, said body having a surface layer integrally united therewith, said layer consisting essentially of an alloy of the metals of said oxides.

6. A magnetostrictive element comprising a ferrospinel body including chemically combined metallic oxides, said body being of the type which exhibits a large magnetostriction upon the application of a magnetic field, said body having a surface portion thereof chemically reduced to metals of said metallic oxides.

7. A magnetostrictive element comprising a ferrospinel body consisting essentially of substantially equimolar proportions of nickel oxide and ferric oxide, in chemically combined form, said body having a surface portion thereof chemically reduced to metals of said oxides.

References Cited in the file of this patent

UNITED STATES PATENTS

|    |           |               |               |
|----|-----------|---------------|---------------|
| 40 | 1,884,665 | Greiner       | Oct. 25, 1932 |
|    | 1,922,254 | McCulloch     | Aug. 15, 1933 |
|    | 2,860,450 | Case          | Nov. 18, 1958 |
|    | 2,957,238 | Harvey et al. | Oct. 25, 1960 |